

# UNITED STATES PATENT OFFICE.

WILBUR B. DRIVER, OF EAST ORANGE, NEW JERSEY.

## CHROMIUM ALLOYS.

1,175,724.

Specification of Letters Patent. Patented Mar. 14, 1916.

No Drawing.

Application filed June 24, 1912. Serial No. 705,442.

To all whom it may concern:

Be it known that I, WILBUR B. DRIVER, a citizen of the United States, and a resident of the city of East Orange, State of New Jersey, (whose post-office address is Middlesex street, Harrison, Newark, New Jersey,) have invented new and useful Chromium Alloys, which invention is fully set forth in the following specification.

10 My invention relates to chromium alloys intended primarily for use as an electrical-resistance element.

15 The purpose of the invention is to produce a novel class of non-oxidizing alloys that are ductile and malleable, with a high electrical-resistance and a low temperature-coefficient.

20 More specifically, a preferred form of my invention is based on the discovery that whereas a substantial percentage (say, five to ten per cent.) of chromium added to copper alone gives such inferior mechanical qualities that the material is practically valueless, yet when the chromium is to be 25 added to a mixture or alloy of copper and some other metal such as manganese or nickel, the chromium may be added in substantial quantities (say, from about ten per cent. to almost twenty per cent.) and yet 30 produce an alloy which is ductile and malleable, and which affords a relatively high resistance to oxidation; moreover, the alloys of this new class present a high electrical resistance and have a low temperature- 35 coefficient, so that they are particularly suitable for electrical-resistance purposes.

Other things being equal, increase in the percentage of chromium increases the resistance to oxidation, but decreases the work- 40 ability of the composition. With as much as twenty per cent. of chromium, the material appears rather difficult to work; but with around ten per cent. of chromium, it works easily, and such ten per cent. chromium alloys are found to be very suitable 45 for electrical-resistance purposes. Even an amount of chromium as low as two per cent. produces a marked effect.

Broadly my invention contemplates an alloy containing chromium, more specifically 50 chromium and copper. I prefer, however,

an alloy comprising chromium and copper with some other metal or metals, and particularly such three-metal alloys in which there is a substantial percentage of the chromium. The preferred amount of chromium is around ten per cent., although the percentage may vary as between, say, two per cent. and twenty per cent.

As one example, take about 45 parts, by weight, of copper, about 45 parts of nickel, and about 10 parts of chromium, and fuse them together in any convenient manner. As another example, take about 50 parts, by weight, of nickel, about 30 parts of copper, about 10 parts of manganese, and about 10 parts of chromium, and fuse them together in any convenient manner. The lowest temperature coefficients have been obtained where the nickel and copper are used 70 in about equal amounts, and as the nickel is increased the alloy becomes harder. But these nickel-copper-chromium alloys, with or without manganese, give very good results, both where the nickel predominates 75 and where the copper predominates. The effect of the addition of chromium to alloys containing nickel and copper, increases as the percentage of the nickel increases. In other words, it seems as though the chromium has a greater effect, for electrical resistance, upon the nickel than upon the copper.

Having thus described my invention, I claim:

1. An electrical-resistance element consisting of an alloy containing copper and nickel and manganese, with from about two per cent. to about ten per cent. (2-10%) of chromium.

2. An electrical-resistance element consisting of an alloy containing copper and nickel and manganese, with a substantial percentage of chromium.

In testimony whereof I have signed this 95 specification in the presence of two subscribing witnesses.

WILBUR B. DRIVER.

Witnesses:

C. A. L. MASSIE,  
RALPH L. SCOTT.